

## UNITED STATES PATENT OFFICE

HERMANN WAGNER, OF SODEN-ON-THE-TAUNUS, AND HEINZ EICHWEDE AND ERICH FISCHER, OF HOCHST-ON-THE-MAIN, GERMANY, ASSIGNEES TO GENERAL ANILINE WORKS, INC., OF NEW YORK, N. Y., A CORPORATION OF DELAWARE

## DYEING MIXED TEXTILE GOODS MADE OF WOOL AND SILK FIBERS

No Drawing. Application filed March 17, 1927, Serial No. 176,298, and in Germany March 22, 1926.

As is known only a few acid azo dyestuffs possess the property of dyeing evenly wool and silk fibers in a single bath. In U. S. Patent 1,678,611, it has been set forth that such pyrazolone azo dyestuffs as contain one or more carboxylic acid ester groups are distinguished by an increased affinity for the silk fiber.

Now we have found that pyrazolone-azo dyestuffs containing one or more of the ether groups—alkyloxy-, aryloxy- and aralkyloxy—are also eminently suitable for producing very even tints on mixed textile goods made of wool and silk fibers.

In the following examples the mark → signifies that the amino body standing before the arrow is diazotized and coupled with the component standing in the direction of the arrow. These examples serve to illustrate our invention but they are not intended to limit it; the parts are by weight:

(1) 1 kg. of a fabric of mixed wool and silk fibers is dyed in an appropriate manner in a dyebath containing 20 g. of the dyestuff: 25 ortho-aminoanisole → 1-(4'-sulfophenyl)-3-methyl-5-pyrazolone, while adding 10% of sodium sulfate and 4% of sulfuric acid. The dyeing thus obtained is not only remarkable for its great general fastness but also for the 30 fact that the wool fibers as well as the silk fibers are dyed evenly and one and the same shade. The dyestuff has the following constitution:



40 (2) By substituting for the dyestuff indicated in Example 1 an equal quantity of the dyestuff: ortho-amino-diphenylether → 1-(4'-sulfophenyl)-3-methyl-5-pyrazolone, 45 there is obtained the same result as in Exam-

ple 1. The dyestuff has the following constitution:



The combinations specified in the foregoing examples may be largely varied both as regards the diazotizing component and the coupling component. It is, however, advantageous to prepare the dyestuff in such a manner that its molecule does not contain more acid groups than are necessary for rendering the dyestuff soluble.

60 Besides the dyestuffs used in Examples 1 and 2 there may also advantageously be used the following dyestuffs:

3-amino-1-methyl-4-phenylbenzylether → 70 1-(4'-sulfophenyl)-3-methyl-5-pyrazolone of the following constitution:



Ortho-aniline-sulfonic acid → 1-(4'-methoxyphenyl)-3-methyl-5-pyrazolone of the following constitution:



90 Para-aminodiphenylether-ortho-sulfonic

acid→1-phenyl-3-methyl-5-pyrazolone of the following constitution:



or the like.

The dyestuffs are prepared in known manner by causing the diazo compounds to act upon the pyrazolones obtainable from the corresponding hydrazines and acetoacetic ester.

The affinity of the dyestuffs for the silk fiber is enhanced if both the diazo component and the coupling component contain one or more of the ether groups—consisting of alkyloxy-, aryloxy- and aralkyloxy—or if one of the components contains an ether group and the other a carboxylic acid ester group. Besides the above-cited monoazo dyestuffs there may also advantageously be used disazo dyestuffs obtained in a suitable manner by synthesis.

In the appended claims the term "ether group" is to be understood as including alkyloxy, aryloxy and aralkyloxy groups.

We claim:

1. The process which comprises dyeing mixed textile goods made of wool and silk fibers with a pyrazolone-azo dyestuff containing both in its diazo component and in its coupling component several ether groups.

2. The process which comprises dyeing mixed textile goods made of wool and silk fibers with a pyrazolone-azo dyestuff containing in one of its two components several ether groups.

3. The process which comprises dyeing mixed textile goods made of wool and silk fibers with a pyrazolone-azo dyestuff containing both in its diazo component and in its coupling component an ether group.

4. The process which comprises dyeing mixed textile goods made of wool and silk fibers with a pyrazolone-azo dyestuff containing in one of its two components an ether group.

5. As new products, mixed wool and silk textile goods dyed with a water-soluble pyrazolone-azo dyestuff containing both in its diazo component and in its coupling component several ether groups.

6. As new products, mixed wool and silk textile goods dyed with a water-soluble pyrazolone-azo dyestuff containing in one of its two components several ether groups.

7. As new products, mixed wool and silk textile goods dyed with a water-soluble pyrazolone-azo dyestuff containing both in its diazo component and in its coupling component an ether group.

8. As new products, mixed wool and silk textile goods dyed with a water-soluble pyrazolone-azo dyestuff containing in one of its two components an ether group.

9. As new products, mixed wool and silk textile goods dyed with a pyrazolone-azo-dyestuff of the following formula:



wherein  $\alpha$  represents a substituent of the group consisting of hydrogen and alkoxy.

10. As new products, mixed wool and silk textile goods dyed with a pyrazolone-azo-dyestuff of the following formula:



11. As new products, mixed wool and silk textile goods dyed with the pyrazolone-azo-dyestuff of the following formula:



In testimony whereof, we affix our signatures.

HERMANN WAGNER.  
HEINZ EICHWEDE.  
ERICH FISCHER.

100

105

110

115

120

125

130